

## UNITED STATES PATENT OFFICE

2,102,799

## PROCESS FOR DEHYDRATING CELLULOSE NITRATE

David G. Kennedy and Joseph Keen Rulon, Parlin, N. J., assignors to E. I. du Pont de Nemours & Company, Wilmington, Del., a corporation of Delaware

No Drawing. Application November 8, 1934,  
Serial No. 752,113

2 Claims. (Cl. 260—148)

This invention relates to an improved process for the removal of water from wet cellulose nitrate and its replacement by alcohol.

In the preparation of cellulose nitrate, raw material such as cotton linters is nitrated and when the nitration is carried to the extent desired, the surplus nitrating acids are removed and the nitrated material is at once drowned in water. The nitrated material is carried away by the drowning water to a vat where boiling is conducted to remove excess acid. Several changes of water are used in this process. The water wet nitrocellulose is then delivered to another operation for water removal.

When the cellulose nitrate is to be used, this water must be removed so that a cellulosic material may be dispersed in solvents with which water is usually incompatible. In the present practice the water is usually replaced by an alcohol which subsequently forms a part of the dispersing medium. One commercial method used at present for the dehydration operation is as follows:

The cellulose nitrate, which contains from 20 to 30% of water, is mixed with four or five times its weight of 95% alcohol and the slurry placed in a centrifuge to remove the excess alcohol. This step is usually repeated until alcohol of a fairly high strength remains in the cellulose nitrate. Ordinarily, the treatment is adjusted so that the cellulose nitrate contains about 30% of its weight of alcohol which runs about 90%.

Another procedure commonly used is one in which a specially adapted hydraulic press is employed. In this procedure the water wet cellulose nitrate is placed in the cylinder of the press, and the material pressed until the press cake contains approximately 30% of water. Alcohol is then forced through the press cake until the water is replaced to the desired extent by the alcohol. Both of these operations are somewhat costly, due to the large amounts of diluted alcohol obtained from the operation. The recovery and rectification of the alcohol in these methods adds greatly to the cost of the process.

This invention has as an object a method which provides for the removal of water from the wet cellulose nitrate in such a manner that less diluted alcohol is obtained. A further object is the provision of a method which reduces the loss of cellulose nitrate, due to its solubility in the dehydrating medium, to a minimum.

These objects are accomplished by treating the wet cellulose nitrate under pressure with diluted alcohol obtained from a previous treatment, fol-

lowed by a second treatment with undiluted alcohol while the press cake is still under pressure. The invention is carried out in its specific embodiment by placing cellulose nitrate after it has been drowned and the surplus water removed by placing it in a hydraulic press and squeezing out most of the water contained in the wet cellulosic material. While the cellulose nitrate is still under pressure, a measured quantity of diluted alcohol is pumped into the press and forced through the press cake, thereby replacing the water which remains in the material.

As the diluted alcohol enters the press cake, the water and some of the alcohol are removed at the same time through the discharge line at the base of the press. Following this treatment with diluted alcohol, a measured quantity of undiluted alcohol is pumped into the press and forced through the press cake, so that the diluted alcohol contained in the cake is replaced by the stronger alcohol. The alcohol thus diluted and part of the stronger alcohol is collected in a measuring tank for re-use as the diluted alcohol described heretofore. This undiluted alcohol is usually 95% strength by volume, and after the diluted alcohol is washed out of the press cake, that which remains is approximately 90% by volume.

The apparatus used may be a hydraulic press of conventional design or it may be specially adapted to the process, as will be apparent to those skilled in the art; for example, the drain valve may be connected by a lever to the inlet valve so that one motion will open both valves at the same time. The position of the measuring tanks, pumps and connecting lines may be placed in any convenient position, as will be readily understood by those familiar with the operation of hydraulic presses.

The process herein disclosed is used for the dehydration of cellulose nitrate as commonly employed in the various arts. As examples, although not limits, of such uses may be mentioned the manufacture of smokeless powder, lacquers of various types, adhesives, plastics, various types of coating compositions for coating fabrics or other non-rigid bases, artificial fibers, photographic and cinema film bases, and other arts where cellulose nitrate is commonly used.

This invention presents as an advantage over the present practice for the dehydration of cellulose nitrate a reduction to about one-half the amount of alcohol used for a given amount of cellulose nitrate. A further advantage is that the use of the diluted alcohol from the second step of

the treatment of one batch of press cake for the first treatment of a subsequent press cake greatly reduces the amount of alcohol which is necessary. The economic aspects of these advantages 5 and the saving in the cost of rectifying smaller quantities of alcohol is readily apparent. A still further advantage in the present invention is the increase in yield of dehydrated cellulose nitrate due to the fact that several types of this material 10 are somewhat soluble in 95% alcohol. Losses occur in the ordinary procedure used at present where undiluted alcohol comes into immediate contact with the cellulose nitrate. This is avoided in the present invention by the use of dilute 15 alcohol in the first treatment. A still further advantage is the amount of cellulose nitrate dissolved in the alcohol having been reduced to a minimum, less alkali is necessary in the subsequent rectification and recovery of the washings. 20 As many apparently widely different embodiments of this invention may be made without departing from the spirit and scope thereof, it is to be understood that we do not limit ourselves to the specific embodiments thereof except as defined in 25 the appended patent claims.

We claim:

1. In the process for preparing cellulose nitrate in which the nitrated cellulose material is

drowned in water and the surplus water removed, the improvement of replacing the remaining water by ethyl alcohol which comprises washing under pressure the wet cellulose material in the form of a press cake first with ethyl alcohol 5 containing a comparatively large amount of water and then with approximately 95% ethyl alcohol until the water in the nitrated cellulose material has been replaced with about 90% alcohol, collecting the diluted alcohol from the second treatment and washing under pressure the original water wet nitrated cellulose with this alcohol in the first stage of a subsequent run. 10

2. The process for removing water from wet cellulose nitrate which comprises treating the 15 water-wet cellulose nitrate under pressure with ethyl alcohol containing a comparatively large amount of water and then washing under pressure the cellulose nitrate with about 95% ethyl alcohol whereby the original water in the cellulose nitrate is replaced by approximately 90% ethyl alcohol, collecting the diluted alcohol from the second treatment, and washing under pressure a fresh mass of cellulose nitrate with the 20 said diluted alcohol as the first stage of the subsequent run. 25

DAVID G. KENNEDY.  
JOSEPH KEEN RULON.